

## UNITED STATES PATENT OFFICE

1,965,012

## PRECIOUS METAL ALLOY COMPOSITION

Norris O. Taylor, Minneapolis, Minn., assignor to  
 Spyco Smelting and Refining Company, Minne-  
 apolis, Minn.

No Drawing. Application May 14, 1934,  
 Serial No. 725,649

1 Claim. (Cl. 75—1)

My invention relates to precious metal alloy compositions. It relates more particularly to compositions of this character for use in wrought and cast dental work and for use in manufacturing jewelry. An object is to produce an alloy which has distinct advantages for such usage.

The full objects and advantages of my invention will appear in connection with the detailed description thereof and the novel features of the invention will be particularly pointed out in the claim.

In carrying out my invention, I utilize as alloy metals, gold, palladium, silver, copper and indium. For the uses above stated, I have found that the different elements may be satisfactorily combined in proportions by weight within the following ranges:

|           | Per cent |
|-----------|----------|
| Gold      | 5 to 15  |
| Palladium | 22 to 30 |

|        | Per cent |
|--------|----------|
| Silver | 37 to 50 |
| Copper | 10 to 20 |
| Indium | ½ to 5   |

Among the advantages of my alloy are the following:

1. It resists oral and atmospheric corrosion.
2. It melts smoothly and casts easily.
3. It is light in weight.
4. It is of pleasing color.

The use of indium is of particular importance in controlling or improving color, corrosion resistance, melting range, hardness, and strength.

I claim:

A precious metal alloy composition composed of from 5 to 15% of gold, from 22 to 30% of palladium, from 37 to 50% of silver, from 10 to 20% of copper, and from ½ to 5% of indium.

NORRIS O. TAYLOR. 75

25

80

30

85

35

90

40

95

45

100

50

105

55

110